

# United States Patent Office.

JOHN B. MELDRUM, OF PATERSON, NEW JERSEY.

*Letters Patent No. 71,034, dated November 19, 1867.*

## IMPROVED FLOOR-CLOTH AND CARPETING.

The Schedule referred to in these Letters Patent and making part of the same.

### TO ALL WHOM IT MAY CONCERN:

Be it known that I, JOHN B. MELDRUM, of Paterson, in the county of Passaic, and State of New Jersey, have invented certain new and useful Improvements in Jute Floor-Cloth or Carpeting, made by printing or stamping in the colors or figures in aniline colors; and I do hereby declare the following to be a full, clear, and exact description of the same.

I take a suitable description of jute-yarns, and bleach them to a white or whitish color by the use of chloride of lime and an alkali, or by other suitable modes. These yarns are woven into a cloth, and on this cloth I print or stamp, by means of blocks or rollers, certain colors, patterns, and designs of aniline colors, which are very bright and durable, or the yarns may be woven into cloth before bleaching, and this cloth, in its grey state, submitted to the bleaching process, and, when bleached, printed, stamped, or ornamented in aniline colors, as above described, and though I prefer the bleached material, the unbleached or grey may be used. The bleaching gives greater brilliancy and permanence to the colors, and enables me to use a greater variety of colors; it causes the coloring matter to strike more deeply into the texture of the cloth, as the fibre is opened up in the process of bleaching, and produces a cloth more pliable and durable than that made without bleaching; but the unbleached material serves a good purpose. The printing of jute cloth in wood colors has been done, but these colors are perishable, and quickly fade out, as they are laid or painted on, and not in, the cloth. Besides, they lack the brightness of the aniline colors. And whilst the bleached jute is preferable, as it makes a better relief or ground for the aniline colors, yet I do not restrict myself to its use alone, as I can use, and make a very good, cheap, and merchantable carpet out of the grey or unbleached jute cloth. I of course use such aniline colors as are made of that substance for the brightest portions of the cloth or carpet, and may use in addition to them such other colors, not procurable from that material, but claim only the use of aniline colors, whether used alone, or whether portions of the cloth or carpet are printed in other colors or not.

Having thus fully described my invention, what I claim as a new article of manufacture, is—  
A jute floor-cloth or carpet printed with aniline colors, substantially as and for the purpose described.

J. B. MELDRUM.

Witnesses:

A. B. STOUGHTON,  
EDM. F. BROWN.